

## 1

2,859,159

**BRIGHT COPPER PLATING BATH CONTAINING MIXTURES OF METAL COMPOUNDS**

Christian J. Wernlund, Niagara Falls, N. Y., assignor, by mesne assignments, to Elechem Corp., Jersey City, N. J., a corporation of New Jersey

No Drawing. Application October 9, 1956  
Serial No. 614,826

6 Claims. (Cl. 204—44)

This invention relates to the production of bright copper electrodeposits from aqueous cyanide solutions containing certain metallic addition agents, antimony in particular.

The present application is a continuation-in-part of my copending application Serial Number 352,268, filed April 30, 1953, now abandoned.

As shown in my U. S. Patent No. 2,774,728, trivalent antimony is especially distinguished as an additive in aqueous copper cyanide plating solutions by its ability to produce brilliant, soft, ductile and readily buffable copper deposits. A disadvantage of the antimony is the narrowness of the current density range within which it can produce the desired bright deposits.

A broad object of this invention is to effect improvements in the electrodeposition of copper from aqueous copper cyanide solutions.

A further object is to effect improvement in the electrodeposition of copper from aqueous cyanide solutions containing a metallic brightening agent.

Another object is to extend the bright plating range of aqueous cyanide solutions containing a metallic brightening agent.

A specific object is to provide an aqueous bath containing copper cyanide and trivalent antimony and possessing an improved bright electroplating range.

The above-mentioned and still further objects are achieved in accordance with this invention by electrodepositing copper from a cyanide bath containing both a primary metallic addition agent, usually antimony, and

## 2

are added. Preferred are potassium baths containing, in aqueous solution:

| 5 | Component                   | Satisfactory Range (oz./gal.) | Preferred Range (oz./gal.) |
|---|-----------------------------|-------------------------------|----------------------------|
|   | Potassium hydroxide.....    | 1-10                          | 1-8                        |
|   | Free potassium cyanide..... | 0.5-4                         | 1-2                        |
|   | Copper cyanide.....         | 5-20                          | 8-14                       |

10 The "free" cyanide is that measured by the liebig silver nitrate titration.

The cheaper sodium compounds are frequently substituted in whole or in part for potassium compounds.

15 Since the potassium formulations permit higher rates of copper deposition and produce slightly brighter deposits, they are technologically preferred.

Antimony, the preferred primary brightener of the invention, may be added to the basic solution in almost any of its soluble trivalent forms. Antimony trioxide, potassium antimonyl tartrate, and many other compounds may alike be used. The quantity of antimony employed may vary between about 0.010 and 0.20 g./l., considered as the metal, with about 0.050 and 0.10 g./l. preferred. 20

25 The weight of the antimony compound supplying this desired weight of antimony may, of course, be readily determined from the appropriate gravimetric factors.

In addition to the preferred antimony, several other metals may serve as the primary brightener of this 30 invention. These metals are bismuth, mercury, silver and cadmium. While they may be supplied as many of their soluble compounds, representative compounds and weights are given in the table below.

35 The secondary brighteners of the invention are zinc, arsenic, cobalt, iron and cadmium. The anomalous appearance of cadmium as both a secondary and a primary brightener is due to the fact that it exhibits improved results when employed with any other member of either of the brightening groups disclosed.

40 The secondary brighteners may also be supplied to the bath in about any convenient soluble compound. Representative compounds and weights are included in the table below along with the same data for the primary brighteners.

TABLE.—CONCENTRATION OF METALLIC BRIGHTENERS WHEN USED IN PAIRS

| Metal         | Weight of Metal   |                   | Compound Added                                                                    | Weight of Compound (g./l.) |
|---------------|-------------------|-------------------|-----------------------------------------------------------------------------------|----------------------------|
|               | Effective (g./l.) | Preferred (g./l.) |                                                                                   |                            |
| Antimony..... | 0.010-0.20        | 0.050-0.10        | KSbO <sub>2</sub> C <sub>4</sub> H <sub>4</sub> O <sub>6</sub> ·½H <sub>2</sub> O | 0.03-0.5                   |
| Bismuth.....  | 0.002-0.05        | 0.002-0.01        | Bi(C <sub>6</sub> H <sub>5</sub> O <sub>6</sub> ) <sub>3</sub> ·7H <sub>2</sub> O | 0.01-0.2                   |
| Mercury.....  | 0.008-1.60        | 0.008-0.08        | Hg(CN) <sub>2</sub>                                                               | 0.01-2.0                   |
| Silver.....   | 0.008-1.62        | 0.008-0.08        | AgCN                                                                              | 0.01-2.0                   |
| Cadmium.....  | 0.007-7.00        | 0.070-3.50        | Cd(CN) <sub>2</sub>                                                               | 0.01-10                    |
| Zinc.....     | 0.056-2.32        | 0.120-1.65        | Zn(CN) <sub>2</sub>                                                               | 0.10-4.0                   |
| Arsenic.....  | 0.760-7.60        | 0.760-3.80        | As <sub>2</sub> O <sub>3</sub>                                                    | 1.00-10.0                  |
| Cobalt.....   | 0.003-0.32        | 0.016-0.16        | K <sub>3</sub> Co(CN) <sub>6</sub>                                                | 0.02-2.0                   |
| Iron.....     | 0.088-0.40        | 0.180-0.36        | K <sub>4</sub> Fe(CN) <sub>6</sub>                                                | 0.50-2.3                   |

also a secondary metallic agent synergistically cooperates with the primary in forming bright copper deposits. The secondary agents of this invention are cobalt, iron, arsenic, cadmium, and zinc.

65 Almost any substantially conventional aqueous copper cyanide plating solution may be employed as the basic baths to which the metallic brighteners of this invention

are added. Preferred are potassium baths containing, in aqueous solution:

The compounds cited in the table as yielding the desired metallic additive are intended as purely illustrative and not as sharply restrictive. In general any compound of the particular additive can be utilized that is compatible with the bath being employed, i. e., is soluble in the bath and does not change important bath characteristics such as the pH. The weight of compound

added will be that necessary to give a weight of the desired metal within the range designated as effective.

The modified baths of this invention, like many cyanide copper baths, may yield rough plate unless precautions are taken thereagainst. Conventional anti-pitting agents are therefore generally also added to the baths. Satisfactory anti-pitting agents are the betaines, e. g., C-decyl betaine, of the type shown by Holt, U. S. Patent 2,255,057.

Operational conditions for the present electroplating process are substantially those of the prior art. Thus a temperature of about 60-95° C. may be employed, about 80° C. being preferred. Agitation as by stirring may be employed. Choice of cathodes or workpieces is optional. The usable current density range is broader than that of unmodified baths, bright copper plate being obtained at up to 60 a./s. f. (amps./ft.<sup>2</sup>) or above in some instances.

There follow some examples which serve to illustrate, but not to limit, the invention in more detail.

#### Example 1

This example shows the synergism of antimony and cobalt in aqueous copper cyanide plating solution.

(a) An aqueous copper plating solution was made up with the following composition: 14 oz./gal. of cuprous cyanide, 1 oz./gal. of free potassium cyanide, 5 oz./gal. of potassium hydroxide, and 0.67 oz./gal. of an anti-pitting agent comprising about 30% by weight of trimethyl benzyl ammonium chloride and 12.5% of C-decyl betaine, the remainder being water.

Plating was carried out from this conventional solution under the following conditions:

|                                         |                                         |
|-----------------------------------------|-----------------------------------------|
| Plating tank                            | 1000 ml. oscillating cathode Hull cell. |
| Cathode area                            | 20 in. <sup>2</sup> .                   |
| Cathode current density<br>(front side) | 30-34 a./s. f.                          |
| Rate of stirring                        | 12 ft./min.                             |
| Temperature                             | 80°±2° C.                               |

No bright plate was obtained from this bath above 10 a./s. f.

(b) To the basic plating solution of (a) were added 5 g./l. of potassium cobaltocyanide, K<sub>4</sub>Co(CN)<sub>6</sub>, and plating carried out as before. Bright copper plate was obtained solely in the 17-25 a./s. f. current density range.

To another sample of the solution of (a) was added 50 p. p. m. of antimony as potassium antimonyl tartrate. In this particular instance bright plate was produced only between 14 and 23 a./s. f.

When plating was accomplished from a sample of the bath of (a) containing the cobaltocyanide and 50 p. p. m. of antimony from the antimonyl tartrate, very bright plate was obtained in the 11-44 a./s. f. range. This plate was noticeably brighter than that obtained with either of the additives alone.

#### Example 2

The runs of Example 1 were substantially repeated except that 15 g./l. of potassium ferrocyanide,



were substituted for the cobaltocyanide. The ferrocyanide alone gave bright plate only in the 22-34 a./s. f. range. When combined with 50 p. p. m. of antimony, very bright plate was obtained from 17 to 45 a./s. f. The plate obtained with the dual additives was, as before, noticeably brighter than that obtained with either alone.

70

75

77

#### Example 3

This example shows the combined effect of antimony and arsenic in copper plating baths.

5 A conventional aqueous copper plating bath was made up containing 14 oz./gal. of cuprous cyanide, 2.0 oz./gal. of free sodium cyanide, 6.0 oz./gal. of free potassium hydroxide, 1.5 oz./gal. of sodium carbonate, and the anti-pitting agent of Example 1. This bath, unmodified, produced no bright copper above 10 a./s. f.

10 A portion of the sodium bath containing 0.025 g./l. of antimony added as potassium antimonyl tartrate showed a very bright plating range between 13 and 21 a./s. f. and a semi-bright to a definite dull range at 25 a./s. f. and above.

15 A bath carrying 0.5 g./l. of arsenic trioxide as the sole metallic additive showed a very bright plating range between 20 and 32 a./s. f., hazy bright between 18 and 20 a./s. f. and dull elsewhere.

20 A bath containing both antimony and arsenic, in the quantities utilized separately, showed a very bright low current density plating range between 8 and 36 a./s. f., a semi-bright range up to 50 a./s. f. and a dull range above 50. The combination of additives therefore produces a 25 single bright plating band acceptable both as regards brightness and current density range.

#### Example 4

30 This example shows the joint effect of cadmium and antimony in copper cyanide baths.

35 Copper was electrodeposited from the basic sodium cyanide bath of Example 3 containing additionally 1.0 g./l. of cadmium cyanide and 0.095 g./l. of antimony trioxide. A bright plating range of 15-44 a./s. f. resulted. Antimony trioxide alone in a sodium cyanide bath gave a bright range of 9-18 a./s. f. Cadmium alone gave bright plate in the 35-52 a./s. f. range.

#### Example 5

40 This example shows the joint effect of zinc and antimony in copper cyanide baths.

45 The experiments of Examples 3 and 4 were substantially repeated with 2.0 g./l. of zinc cyanide and 0.050 g./l. of antimony trioxide as the additives. Bright plate was produced in the 9-38 a./s. f. range. Zinc cyanide additive alone gave bright plating ranges of 26-40 and 50-60 a./s. f. Antimony trioxide alone gave a bright range of 9-18 a./s. f.

50 The embodiments of the invention in which an exclusive property or privilege is claimed are defined as follows:

55 1. An aqueous bath for electrodepositing bright copper containing about 5-20 oz./gal. of copper cyanide, about 0.010-0.20 g./l. of trivalent antimony supplied as a soluble salt thereof, and a metal chosen, in the respective proportions specified, from the group consisting of: 0.056-2.32 g./l. of zinc, 0.760-7.60 g./l. of arsenic, 0.003-0.32 g./l. of cobalt, 0.088-0.40 g./l. of iron, and 0.007-7.00 g./l. of cadmium.

60 2. An aqueous bath for electrodepositing bright copper containing about 5-20 oz./gal. of copper cyanide, about 0.010-0.20 g./l. of trivalent antimony supplied as a soluble salt thereof, and about 0.120-1.65 g./l. of zinc.

65 3. An aqueous bath for electrodepositing bright copper containing about 5-20 oz./gal. of copper cyanide, about 0.010-0.20 g./l. of trivalent antimony supplied as a soluble salt thereof, and about 0.760-3.80 g./l. of arsenic.

70 4. An aqueous bath for electrodepositing bright copper containing about 5-20 oz./gal. of copper cyanide, about 0.010-0.20 g./l. of trivalent antimony supplied as a soluble salt thereof and about 0.016-0.16 g./l. of cobalt.

75 5. An aqueous bath for electrodepositing bright copper containing about 5-20 oz./gal. of copper cyanide, about

0.010-0.20 g./l. of trivalent antimony supplied as a soluble salt thereof, and about 0.180-0.36 g./l. of iron.

6. An aqueous bath for electrodepositing bright copper containing about 5-20 oz./gal. of copper cyanide, about 0.010-0.20 g./l. of trivalent antimony supplied as a soluble salt thereof, and about 0.070-3.50 g./l. of cadmium. 5

References Cited in the file of this patent

UNITED STATES PATENTS

1,120,794 Daft Dec. 15, 1914 10

1,120,795 Daft Dec. 15, 1914  
1,559,077 Latre et al. Oct. 27, 1925  
2,737,485 Overcash et al. Mar. 6, 1956

OTHER REFERENCES

Ernst et al.: Transactions Electrochemical Soc., vol. 61 (1932), pp. 363, 391-394.